

## UNITED STATES PATENT OFFICE

2,448,037

## LUBRICATING COMPOSITIONS

Bert H. Lincoln, Ponca City, and Gordon D. Byrkit, Niagara Falls, N. Y., assignors, by mesne assignments, to The Lubri-Zol Development Corporation, Cleveland, Ohio, a corporation of Delaware

No Drawing. Application December 8, 1944,  
Serial No. 567,304

14 Claims. (Cl. 252—33.6)

1

This invention relates to lubricating oils and more particularly to improved lubricating oils of high film strength, high resistance to oxidation, and markedly reduced formation of corrosive products during use.

Present-day mechanical devices require lubricating oils of high film strength, of high oiliness characteristics, and of low tendency to oxidize during use. It has been found that the present-day hydrocarbon lubricants of the very highest quality are deficient in these very important characteristics. These three properties are of vital importance under conditions of thin film lubrication where the lubricant has been squeezed from between the friction surfaces because of high pressure, slow speeds, and other causes. In modern engines, large surfaces of oil are exposed to the action of atmospheric oxygen, promoting rapid oxidation. It is readily seen that the viscosity or the body of the lubricant plays no part in thin film lubrication and that the remaining film of oil must have a very high film strength and be of high oiliness value to prevent rupture of the film of the lubricant, which would cause seizure. The oil film must tend to keep the coefficient of friction as low as possible. The oil must resist oxidation when these thin film are heated in the presence of atmospheric oxygen as they are in use.

Mechanical devices are being designed for higher pressure operation, and the film strength of the best quality straight hydrocarbon lubricant has been found to be too low for satisfactory service. It will be obvious that an invention which provides a means of improving the film strength of these lubricants is of great importance to the art of lubricant manufacture and to the designer and fabricator of mechanical devices.

Substantially all machines operate in part or at times totally under conditions of boundary or thin film lubrication, under which conditions the oiliness or unctuousness of the lubricant is the first and primary requisite of efficient operation. Those skilled in the art of lubricant manufacture or machine manufacture will readily appreciate the value of an invention that will improve the oiliness of these otherwise high-quality lubricants. Furthermore, sludge and acid are especially deleterious under conditions of thin film lubrication. The sludge is not a lubricant in any sense of the word, and the soluble acid is particularly corrosive to bearing metals such as cadmium-silver, copper-lead, and the like.

In starting idle mechanical equipment which

2

is lubricated from a sump by pumping or circulating the lubricant, there is always a short period of time in which the rubbing surfaces must operate under conditions of dry friction if ordinary hydrocarbon lubricants are used. With dry friction, the wear on friction surfaces is extreme; and during cold weather when the lubricant is sluggish or during periods when the lubricating system is not functioning properly for one reason or another, rubbing surfaces may not only suffer considerable wear but may be damaged to the point where they must be replaced. The product of our invention has a very important property of reacting with the metal surfaces, penetrating or adsorbing on the metal surfaces, and leaving a film of lubricant with high oiliness character, which remains on the metal surface irrespective of the length of time the machine has been idle.

20 This high oiliness film gives very even and smooth operation, which may be easily discerned by the experienced operator or lubricating engineer.

When the hydrocarbon lubricants are diluted 25 with unburned fuel or with other light hydrocarbons, the small degree of oiliness of the original hydrocarbon lubricant is greatly decreased. We have found that the addition of the products of our invention to hydrocarbon lubricants more than compensates for the loss in oiliness and load-carrying ability from dilution.

It is well known that, in order to obtain lubricants which are preeminently satisfactory from the standpoint of oxidation in use, it is necessary to refine the oil thoroughly and then to add 35 an inhibitor of oxidation. The thorough refining may consist of more and heavier acid treatments or solvent treating so as to remove a considerable part of the oil and leave only the most stable portion. Such drastic refining is necessary in order to obtain stability with respect to sludge formation, but the oil is then subject to easy oxidation to form soluble acids and other corrosive materials. This can be prevented by the addition to the refined oil of small amounts of materials which either prevent the formation of these corrosive products or by some action render them inert. Furthermore, such well-refined oils are susceptible to the formation 45 during use of lacquer-like materials which tend to stick rings. This results in blow-by and hence loss of power, failure of lubrication, scratching, scoring, overheating, and eventually replacement of parts. It is practically impossible to refine a lubricant in such a manner as to avoid all three

of these difficulties, namely, soluble corrosive products, sludge, and lacquer. It is considerably more advantageous to add the materials of our invention and avoid these difficulties by this method.

Certain compounds are adsorbed or absorbed by metals thus forming tenacious films at the surface of metals; these films are able to stand high pressures. X-ray diffraction methods have shown that compounds containing highly polar molecules, that is molecules of unsymmetrical electrical character containing an atom or group of atoms exhibiting a secondary or residual valence, tend to produce regimentation of the molecules of hydrocarbon oil when added thereto. A metal immersed in a strongly polar compound will show a film of the compound in which there is a regimentation of molecules oriented with respect to the surface of the metal by which they are adsorbed or absorbed.

Many of our additive materials are effective when added to poorly refined or even wholly unrefined lubricants. The addends may thus be substituted in whole or in part for the usual refining processes.

In the prior art of applying these principles to the manufacture of lubricants, many diverse types of materials have been suggested to be added to obtain improvement in various characteristics. It has been found that the addition of various compounds frequently improves film strength, oxidation resistance, noncorrosiveness, and other characteristics.

One object of our invention is to provide improved inhibitors of oxidation and corrosion for addition to lubricants.

Another object of our invention is to provide film strength improving addition agents suitable for use in lubricants and especially in crankcase lubricants.

A further object of our invention is to provide a lubricant having detergent properties in addition to the above.

Other and further objects of our invention will appear in the course of the following description.

To the accomplishment of the foregoing and related ends, said invention, then, consists of the means hereinafter fully described and particularly pointed out in the claims.

In general, our invention contemplates an oil of lubricating viscosity having added thereto a small amount of an organic thiocarbonate of the general formula



in which C represents carbon, X represents either oxygen or sulphur (at least one of the X's must be sulphur) and R and R' are organic radicles one or both of which contain carbon, hydrogen, and at least one other element besides halogen. Halogen may be present in the R's but in that case another characterizing element must also be present. The elements which we refer to here as "characterizing elements" include oxygen, sulphur, selenium, nitrogen, phosphorus, and metallic elements such as tin, arsenic, antimony, bismuth, aluminum, calcium, barium, magnesium, sodium, lithium, and the like. The R's may be aliphatic, carbocyclic, or heterocyclic in character. It will be apparent that by thiocarbonate in the appended claims we mean to include mono- and tri-thiocarbonates as well as the di-thiocarbonates (xanthates).

The introduction of this characterizing element or elements into our thiocarbonates permits of an extraordinary flexibility in the design of the addend for a particular use.

Thus it permits the introduction of additional oxygen or sulphur in such active forms as, for example, halogenated carboxylic or thio-carboxylic acids, their esters, metal salts, ammonia, amine, or aniline salts, as shown in the following type formula:



in which the substituted thiocarbonate radicle is as described above wherein, however, R's is further defined as an organic radicle containing:

Y—a halogen, preferably in the alpha or adjacent position to a carbon atom having the  $>C=X$  group,

20 X—the element oxygen or sulphur,

R—an organic radicle preferably:

- an alkyl radicle of from 11 to 15 carbon atoms,
- an aryl radicle such as phenyl, phenoxy-phenyl, naphthyl etc.
- an alkylated aryl radicle such as o, p-di-iso-amylophenyl cresyl, 2,4-di-methylnaphthyl, etc.

25 and Q—is a radicle selected from the group consisting of R; M, M'R, M"R, etc.; M'-OR, M'-O—O—C—R, etc.; NH<sub>2</sub>, NH<sub>3</sub>R, NH<sub>2</sub>R<sub>2</sub>, etc.; AsR<sub>3</sub>, PR<sub>3</sub> etc. where M is a monovalent metal, M' is a divalent metal, and M" is a trivalent metal.

It is clear, from the above type formula, that 30 the neutralized halogenated xanthated esters or salts of alkyl, arylalkyl, or alkylated arylalkyl fatty acids are among the preferred forms of the additive.

In compounds of this type, we introduce additional active groups beyond the thiocarbonates 35 previously described; thus by the use of halogenated fatty acid esters, we introduce high oiliness and load-carrying capacity beyond that obtainable from the thiocarbonates or xanthates alone.

40 Similarly, by the use of halogenated fatty acid or arylated fatty acid metal salts, we introduce detergency not otherwise obtainable from the thiocarbonates or xanthates alone.

Compounds illustrative of these oxygen or sulphur containing halogen substituted thiocarbonates are:

1. Methyl ethylxanthyl-chlorostearate
2. Barium ethylxanthyl-chlorostearate
3. Calcium amyloxanthyl-phenyl chlorostearate
4. Tin butylxanthyl-p-chlorophenyl chloroacetate
5. Lithium ethylxanthyl-o,p-di-isoamylphenyl chloroacetate
6. Thiophenyl ethylxanthyl-chlorostearate
7. Barium amyloxanthyl-naphthyl chloromonothioacetate

The additional inhibiting action of phosphorus, 55 nitrogen, or other inhibiting groups may be added to the molecule to produce an extremely effective inhibitor of oxidation and/or corrosion.

Thus nitrogen and/or phosphorus may be introduced as the salt-type compound of the thiocarbonate substituted halogenated fatty acids described above or as otherwise substituted in the molecule. For example, when nitrogen is present in the molecule, it may be present in combination with the halogenated aliphatic or aryl-aliphatic acid as:

65 a. Amide, anilide, hydrazide, etc.



70 where X, Y, and R are as defined above, and Q' is a nitrogen containing radicle selected from the group consisting of simple or substituted nitrogen, e.g. NH<sub>2</sub>, NH<sub>3</sub>R, NR<sub>2</sub>, NH—NH<sub>2</sub>,



etc., having R groups of alkyl, aryl, cycloalkyl, or heterocyclic nature.

## b. Ammonium salts



where X, Y, and R are as defined above, and Q'' is a nitrogen containing radicle selected from the group consisting of simple or substituted nitrogen salts, e.g., NH, NH<sub>2</sub>R, NH<sub>2</sub>R<sub>2</sub>, etc., having R groups of alkyl, aryl, cycloalkyl, or heterocyclic nature.

c. Other salt-type compounds of the xanthated, halogenated acid and nitrogen bases such as pyridine, quinoline, nitrogen bases from coal tar or petroleum fractions, natural alkaloids, and the like.

The newly introduced element or elements in addition to halogen have a considerable effect on the activity of the thiocarbonate sulphur and it may be activated or depressed by the use of suitable groups in the R's of our thiocarbonates. Chlorine may in turn have an activating effect on the characterizing element or elements.

The substituted thiocarbonates of our invention show an unexpected improvement over the corresponding unsubstituted thiocarbonates and even over mixtures of the unsubstituted thiocarbonates with other compounds having the same substituting groups. Thus a xanthate containing a chlorostearic acid ester group shows a greater effect as an oiliness agent than the chlorostearate group in, say, methyl chlorostearate plus the same xanthate without the chlorostearate group. Similar unexpected results are obtained on the introduction of metal salts as a detergency factor in addition to halogen, oxygen and/or sulphur and the like as film strength or inhibiting factors.

The particular thiocarbonates of this invention have a multiple action in a lubricant. One action involves increased load-carrying ability and/or oiliness, while other actions are directed to detergency and the stability of the lubricant. For load-carrying capacity, quantities ranging from 0.1 per cent to about 10 per cent may be added. As an anti-corrosive agent and/or an anti-sludging agent, much smaller amounts may be required ranging from approximately 0.001 to 1.0 per cent. The action of our thiocarbonates is specific but difficult to understand. These compounds may be added to any type of hydrocarbon lubricants but show an unusual value in highly refined and solvent treated lubricants. By oil having lubricating viscosity in the appended claims, we mean to include the so-called mineral oils and various hydrogenated, polymerized and otherwise synthetically treated oils such as volatilized oils, aluminum chloride treated oils, and the like. Furthermore the lubricating oil may consist in whole or in part of shale oil, animal or vegetable oils such as castor oil, lard oil, corn oil, cottonseed oil, and the like.

In practice, it is better to employ compounds whose boiling point is above 225° F. in order that the addition compound will not be evaporated or distilled in use. The selection of a particular compound or compounds to be used as an addition agent to the hydrocarbon or other oil is to be made considering the physical and chemical properties of the various compounds and the use to which the blend is put. Thus, if water is likely to be present during use, a salt or combination of salts is selected which is not affected by water. If a particular added compound proves too volatile for its application, a higher boiling material should be used and the more volatile compound used for blending in an oil intended for duty at lower temperatures. In general, for automotive crankcase lubricants, we prefer to use com-

6 pounds having vapor pressures of less than atmospheric at 250° F.

The following compounds may be used in accordance with our invention. All and each of these are to be considered as examples of our invention when blended in minor proportion in an oil of lubricating viscosity. One or both of the organic radicles in our mono-, di-, or tri-thiocarbonates may be of various types as shown in the following classification. Each of the following organic, or organo-metallic radicles may be combined with mono-, di- and tri-thiocarbonate radicles as further examples of our invention.

## I. Aliphatic types

## A. Containing oxygen

## a. Alcohols

1. Hydroxyethyl ethylxanthate
2. Reaction product of potassium laurylxanthate and glycerol monochlorhydrin or glycerol dichlorhydrin
3. Reaction product of potassium ethoxyethylxanthate with chlorinated, hydroxylated paraffin wax which has been chlorinated to 20 per cent chlorine and had half the chlorine removed by treatment with aqueous caustic under pressure to form the hydroxy compound

## b. Ethers

4. Butoxyethyl butoxyethylxanthate
5. Reaction product of potassium amyltrithiocarbonate with paraffin wax chlorinated to 23 per cent chlorine and treated with sodium butylate to remove about one-third of the chlorine to make the butyl ether
6. Reaction product of potassium amylxanthate with beta, beta prime-dichloroethyl ether.
7. Methyl ethoxyamylxanthate

## c. Ketones

8. Reaction product of potassium amylxanthate with chloroacetone
9. Reaction product of potassium amylxanthate with symmetrical dichloroacetone so as to form di(amylxanthymethyl)ketone
10. Reaction product of potassium amylxanthate with symmetrical dichloroacetone so as to form amylxanthymethyl chloromethyl ketone
11. Unsaponifiable oxidation products of paraffin wax chlorinated and part of the chlorine removed by condensation with sodium ethylxanthate

## d. Aldehydes

12. Alpha-butylylxythylbutyraldehyde
13. Alpha-ethoxyethylxanthylloenthaldehyde

## e. Acids and salts

14. Alpha-amylxanthylchlorostearic acid
15. Calcium amylxanthylchlorostearate
16. Tin amylxanthylchlorostearate
17. Ethoxyethylxanthylphenylchlorostearic acid
18. Aluminum ethoxyethylxanthylphenylchlorostearate

## f. Esters

19. n-Butyl ethylxanthylchloroacetate. A mixture of 65 parts of finely powdered potassium ethylxanthate, 65 parts of n-butyl chloroacetate, and 200 parts of acetone was agitated and heated for five hours. The acetone solution was drawn off, concentrated, and the residual oil distilled at 128-135 at one mm. pressure. The product was then halogenated to produce the halogenated additive.

20. Methyl ethylxanthylchlorostearate. A mixture of 48 parts of finely powdered potassium ethylxanthate, 102.5 parts of methyl dichlorostearate, and 100 parts of acetone was similarly refluxed and separated. The residual oil contained 4.05 per cent sulphur. A one per cent blend of this material in a SAE 30 mineral oil showed a Timken film strength of 28 pounds on the arm. The mineral oil alone had a Timken film strength of only 8 pounds on the arm.

## g. Amides

21. Amylxanthylchloro-succindiamide
22. Laurylxanthylchloro-lauramide

## B. Containing sulphur

## a. Mercaptans

23. Mercaptopyanyl butoxyethoxyethylxanthate
24. Amylxanthyl mercaptomethylchlorostearate

## b. Sulphides and polysulphides

25. Reaction product of sodium laurylxanthate with beta, beta prime-dichloroethyl sulphide
26. Reaction product of sodium amyltrithiocarbonate with dichloromethyl trisulphide

## c. Thioacids and derivatives

27. Reaction product of sodium amylmonothiocarbonate with methyl alpha di-chlorothiostearate
28. Reaction product of lithium isobutylxanthate with alpha di-bromothiobutylamide

## d. Sulfones and sulfoxides

29. Reaction product of sodium ethoxyethylxanthate with omega-chloroamylsulfone
30. Reaction product of sodium hexylxanthate with omega-chloroamylsulfoxide

## e. Sulfurized aliphatic compounds

31. Reaction product of potassium hexylxanthate with sulphur- and chlorine-bearing methyl oleate
32. Reaction product of potassium ethylxanthate with sulphur chloride treated methyl linoleate

33. Reaction product of potassium benzylxanthate with sulphur chloride treated methyl esters of soy bean or corn oil acids

- C. Containing nitrogen
- a. Amines
    - 34. Beta-aminochloroethyl ethylxanthate
    - 35. Reaction product of potassium octadecylxanthate with 3-amino-2-chloropentane
    - 36. Reaction product of potassium amylixanthate with 3-dimethylamino-2-chloropentane
  - b. Nitro compounds
    - 37. Omega-nitroamyl amylixanthate
    - 38. Reaction product of potassium butylxanthate with nitro-chloro-paraffin wax
  - c. Cyanides, isocyanides, thiocyanides, cyanates
    - 39. Thiocyanato-ethyl laurylxanthate
    - 40. Reaction product of sodium ethoxyethylxanthate with dichloroacetonitrile
    - 41. Reaction product of sodium propylxanthate with omega-chloroamyl isocyanide
    - 42. Reaction product of sodium amylixanthate with omega-chloroamyl cyanate
  - D. Containing phosphorus
    - 43. Tri(ethoxyethylxanthyl)phosphate
    - 44. Tri(ethoxyethylxanthyl)phosphite
    - 45. Tri(ethoxyethylxanthyl)thiophosphate
    - 46. Methyl butoxyethylxanthyl phosphinochlorostearate
    - 47. Diethylphosphinoethyl amylixanthate
  - E. Containing metals
    - a. Group IV
      - 48. Triethylstannylamyl amylixanthate
      - 49. Triethylplumbylethyl amylixanthylcarbonate
      - 50. Triamylstannylethylxanthylcarbonate
    - b. Group V
      - 51. Diethylarsenylamyl ethylxanthate
      - 52. Diethylantimonyamyl ethylmonothiocarbonate
      - 53. Diethylbismuthylamyl ethylxanthate
    - c. Group VI
      - 54. Amylseleniummethyl ethoxyethylxanthate
      - 55. Amytelluriummethyl butylxanthate
  - II. Carbocyclic types
  - A. Containing oxygen
    - a. Phenols
      - 56. Hydroxyphenyl ethylxanthate
      - 57. Omega-Hydroxyphenylamyl amylixanthate
      - 58. Reaction product of potassium amylixanthate with chlororesorcinol
      - 59. Reaction product of potassium amylixanthate with halogenated paraffin wax substituted phenol
    - b. Alcohols
      - 60. Reaction product of sodium butoxyethylxanthate with o-chlorobenzyl alcohol
      - 61. Reaction product of sodium butylxanthate with hydroxylated, halogenated phenylated wax
    - c. Ethers
      - 62. Anisyl laurylxanthate
      - 63. Omega-phenoxymethyl amylixanthate
      - 64. Phenoxymethyl laurylxanthate
      - 65. Reaction product of potassium benzylxanthate with dichlororesorcinol dimethyl ether
    - d. Ketones
      - 66. Reaction product of sodium ethylxanthate with dichlorobenzophenone
      - 67. Omega-amylixanthylchloracetophenone
      - 68. Reaction product of potassium isobutylixanthate with dichlorostearoylterinalin
    - e. Aldehydes
      - 69. Reaction product of sodium benzylxanthate with o,p-dichlorobenzaldehyde
      - 70. Reaction product of sodium ethoxyethylxanthate with omega-chlorotoluualdehyde
    - f. Acids and salts
      - 71. Reaction product of potassium amylixanthate with cinnamic acid dichloride
      - 72. Reaction product of sodium ethylxanthate with chlorine-bearing dinaphthylstearic acid
      - 73. Calcium salt of the reaction product of sodium laurylxanthate with o,p-dichlorobenzoylbenzoic acid
    - g. Esters
      - 74. Reaction product of potassium amylixanthate and chlorinated phenyl benzoate
      - 75. Phenyl ethoxyethylxanthyl phenylchlorostearate
      - 76. Chlorinated wax condensed (Friedel-Crafts) with phenyl benzoate and sodium amylixanthate
    - h. Amides
      - 77. Potassium butoxyethylxanthate condensed with dichloro-stearamide
      - 78. Amylixanthylchlorosteartoluuidide
    - B. Containing sulfur
      - a. Mercaptans and thiophenols
        - 79. Mercapto-dodecahydro-diphenyl ethylxanthate
        - 80. Reaction product of potassium butyl-monothiocarbonate and o,p-dichlorophenyl ethylmercaptan
      - b. Sulfides and polysulfides
        - 81. Reaction product of dichlorobenzyl disulfide and potassium hexyltrithiocarbonate
        - 82. Reaction product of sodium amylixanthylcarbonate and dichlorophenylethyl disulfide
        - 83. Reaction product of sodium amylixanthylcarbonate with dichlorodiphenyltrisulfide
        - 84. Reaction product of potassium amylixanthate with dichlorodiphenylsulfide
      - c. Thioacids and derivatives
        - 85. Reaction product of sodium laurylxanthate with omega-dichlorothiobutolic acid
        - 86. Reaction product of sodium benzylxanthate with alpha-dichlorothiobutyramide
      - d. Sulfones and sulfoxides
        - 87. Reaction product of potassium octadecylxanthate with dichlorodiphenylsulfone
        - 88. Reaction product of potassium ethyltrithiocarbonate with dichlorodibenzylsulfone
        - 89. Reaction product of sodium ethylmonothiocarbonate with dichlorodibenzylsulfone

- C. Containing nitrogen
- a. Amines
    - 90. Reaction product of lithium butylxanthate with dichlorodiphenylamine
    - 91. Reaction product of sodium benzylxanthate with o,p-dichlorodimethylaniline
  - b. Nitro compounds
    - 92. Nitrocresyl thiocarbonate
    - 93. Amyl nitrobenzylxanthate
  - c. Azo compounds
    - 94. Reaction product of potassium amylixanthate with the product of coupling diazotized o,p-dichloroaniline with alpha-naphthol
  - D. Containing phosphorus
    - 95. Reaction product of sodium ethoxyethyl trithiocarbonate with chlorophosphazobenzene
    - 96. Reaction product of sodium butoxyethoxyethylxanthate with p-chlorophosphinobenzene
  - E. Containing metals
    - 97. Reaction product of triphenyl-omega-dichloroamyl with sodium amylixanthylcarbone
    - 98. Triethylstannyl p-chlorophenyl-benzylxanthate
    - 99. Triethylplumbyl p-chlorophenyl-amylixanthate
    - 100. Ethylmercurio-*o*-chlorophenyl amylixanthate
  - III. Heterocyclic types
  - A. Containing oxygen
    - 101. Reaction product of potassium butylxanthate with polychlorodioxane
    - 102. Reaction product of potassium ethylxanthate with dichlorodiphenylene oxide
    - 103. Reaction product of dichlorohydroxyethyliphene with sodium butoxyethylxanthate
  - B. Containing sulfur
    - 104. Reaction product of potassium ethoxyethylxanthate with chlorothianthrene
  - C. Containing nitrogen
    - 105. Reaction product of potassium amylixanthate with polychloropyridine

When the end-product contains no halogen, or when the end-product contains less than one atom of chlorine per molecule the product may be subsequently halogenated to preferably contain not less than one atom of chlorine per molecule.

Any of these compounds or other members of the classes represented may be used within the scope of our invention.

35 The thiocarbonates have varying degrees of solubility in hydrocarbon and other oils. In some cases it is necessary to use a solvent for the compound or to form colloidal suspensions of the compound in oil. While some of these compounds have only limited solubility in hydrocarbon oils, it is to be remembered that because of their great efficiency extremely small amounts are often effective. Thus we may use as little as 0.001 per cent of some of these compounds, and it will be seen that a fairly insoluble material may dissolve to a sufficient extent to be satisfactory for our purpose. In general, more than 0.001 per cent of our addition agents are used, and we may add one, two, or even five percent or more.

40 Furthermore, it is well known that different types of oils have different capabilities of dissolving a given material. For some purposes, therefore, we prefer paraffinic, for other purposes, asphaltic, and for still other purposes naphthenic or mixed base lubricants. Another method of obtaining a satisfactory mixture of addition agent with the hydrocarbon oil is the use of a mutual solvent to bring the addend into solution. Alternatively, peptizing agents may be added to maintain the thiocarbonates in permanent suspension.

45 Many of the more difficultly soluble materials are rendered more soluble by the introduction of alkyl groups, particularly those containing four or more carbon atoms. The isoamyl, octyl, lauryl, and octadecyl radicals and radicals from paraffin wax greatly increase the solubility of organic compounds in oil. One or more of such groups may be introduced as required.

50 It is sometimes advantageous to combine more than one of these compounds in a blend to obtain particular properties. We accomplish this by mixing two or more of these compounds together and blending the mixture with the hydrocarbon oil or by blending one in the hydrocarbon

oil, blending the second into this mixture, and so on until the composition is complete.

The various thiocarbonates usually improve both the film strength and oxidation characteristics of the hydrocarbon oil. For example, the sludging tendencies may be decreased by as little as 0.001 per cent of our thiocarbonates. The oxidation characteristics of lubricants are very important, and these are markedly improved by our compounds. The ability to reduce friction is another feature contributed to lubricants by some of our compounds.

It may be desirable to include in one and the same blend, in addition to the addends here described, other addends for specific purposes. Thus, we may add a pour point depressor such as a naphthalenechlor wax condensation product, a viscosity index improver such as certain resins or polymerized hydrocarbons, and sulfur or phosphorus containing inhibitors, such as alkyl and aryl phosphate esters in addition to our thiocarbonates. Furthermore, various metallic compounds may be added to the blend without interfering with the action of our ingredients. Indeed, in some cases it is advantageous to combine with our compounds in a hydrocarbon oil blend such materials as calcium dichlorstearate, sodium stearate, sodium oleate, sodium chlorooleate, tin oleate, sodium naphthenates, tin naphthenate, chromium oleate, aluminum stearate, and other metallic soaps or inorganic-organic salts.

Our invention also contemplates the use in lubricating compositions comprising a major proportion of lubricating oil of minor amounts of the previously identified sulphur compounds with a separate organic halogen compound. The halogen compounds which may thus be employed may be classified as follows:

Cyclic compounds, such as halogenated:

I. Benzene and related compounds such as:

(1) Halogenated benzene, e. g.  
(a) chlorinated benzene, e. g.  
the dichlorbenzenes, notably the ortho compound

(b) brominated benzene, e. g.  
ortho-dibrom benzene

(c) fluorinated benzene

(2) Halogenated derivatives of benzene such as:

(a) Halogenated homologs of benzene, e. g.  
mono-chlor toluene

mono-chlor xylene

mono-chlor cyclohexene

ethyl mono-chlor benzenes

propyl mono-chlor benzenes

di-ethyl dichlor benzenes

propyl dichlor benzenes

di-ethyl tetrachlor benzenes

(b) Halogenated amino derivatives of benzene, e. g.

chlorinated aniline

mono-chlor aniline (preferably the ortho compound)

mono-chlor di-methyl aniline

chlorinated toluidines

chlorinated xylydines

chlorinated diphenylamine

(c) Halogenated hydrobenzenes, e. g.  
hydrogenated dichlor-benzenes dichlorhexahydrobenzene (dichlor cyclohexane)

II. Polyphenyls, and related compounds, including diphenyl, diphenyl benzenes, etc., such as:

(1) Halogenated diphenyl, e. g.  
(a) Chlorinated diphenyl, e. g.

mono-chlor diphenyls

di-chlor diphenyls

tri-chlor diphenyls

(b) Brominated diphenyl, e. g.

the mono-brom diphenyls

(c) Fluorinated diphenyl

(2) Halogenated derivatives of diphenyl, such as:

(a) Halogenated homologs of diphenyl, e. g.

chlorinated phenyl-toluenes

ethylated, or propylated, chlorinated

diphenyl, e. g. di-ethyl tetrachlor diphenyl

(b) Halogenated amino derivatives of diphenyl e. g.

chlorinated phenyl-anilines

chlorinated diphenyl amines (xenyl amines)

(c) Halogenated hydrodiphenyls, e. g.

chlorinated phenyl hexahydrobenzene

chlorinated dodecahydrodiphenyl

75

III. Naphthalene and related compounds, such as:

(1) Halogenated naphthalene

(a) Chlorinated naphthalene, e. g.

mono-chlor naphthalene

(b) Brominated naphthalenes, e. g.

mono-brom naphthalene

(c) Fluorinated naphthalene

(2) Halogenated derivatives of naphthalenes, such as:

(a) Halogenated homologs of naphthalenes, e. g.

chlorinated methyl naphthalenes, such as methyl

naphthalene

(b) Halogenated amino derivatives of naphthalene, e. g.

chlorinated naphthylamines

mono-chlor naphthyl amine

(c) Halogenated hydronaphthalenes, e. g.

chlorinated decahydronaphthalene

chlorinated tetrahydronaphthalene

IV. Phenanthrene and anthracene and related compounds, such as:

(1) Chlorinated phenanthrene, chlorinated anthracene

(2) Halogenated derivatives of phenanthrene and anthracene, such as:

(a) Halogenated homologs, e. g.

chlorinated 1-methyl phenanthrene

chlorinated 3-methyl phenanthrene

chlorinated 9,10 dimethyl phenanthrene

chlorinated propyl and isopropyl

derivatives of phenanthrene such as retene

chlorinated dimethyl anthracenes

chlorinated-methyl anthracene

chlorinated propyl and isopropyl derivatives of anthracene

(b) Halogenated amino derivatives, e. g.

chlorinated phenanthryl amines

chlorinated anthramines

(c) Halogenated hydrophenanthrenes and halogenated

hydroanthracenes, e. g.:

chlorinated retene oil (contains hydro retene)

V. Chrysene, picene, and related compounds, including their derivatives, such as homologs, amino derivatives and other substitution products.

VI. Bridged ring compounds, such as the terpenes and related compounds, and their derivatives, e. g. chlorinated pinene.

VII. Heterocyclic compounds, such as pyridine, quinoline, pyrrole thiophene, and derivatives of them, e. g. mono-chlor pyridine.

VIII. Nitriles derived from any of the above compounds, e. g.

Chlorinated:

benzonitrile

toluonitrile

benzyl cyanide

naphthyl cyanide

xenyl cyanide

cyclohexyl cyanide

IX. Sulphides derived from any of the above compounds, e. g.

Chlorinated:

diphenyl sulphide

dibenzyl sulphide

dirxyl sulphides

di-naphthyl sulphides

dixenyl sulphides

dicyclohexyl sulphide

X. Mercaptans derived from any of the above compounds, e. g.

Chlorinated:

benzyl mercaptan

phenyl benzyl mercaptans

naphthyl mercaptans

phenyl propyl mercaptans

cyclohexyl mercaptan

XI. Thiocyanates, e. g.

Chlorinated:

benzyl thiocyanate

phenyl ethyl thiocyanate

phenyl propyl thiocyanate

cyclohexyl thiocyanate

Halogen-bearing aliphatic compounds:

I. Hydrocarbons, e. g.

Chlorinated or fluorinated hydrocarbons which contain from four to ten or more carbon atoms and certain others containing less than four carbon atoms, e. g.

hexachlor ethane

pentachlor ethane

chlor propane

chlor butane

chlor pentane

fluor hexane

fluor octane

fluor decane

tetrachlor ethylene

hexachlor propylene

chlor butylenes

chlor pentenes

chlorinated unsaturated hydrocarbons obtained from products of partial pyrolytic decomposition of high boiling petroleum hydrocarbons.

chlorinated petroleum wax

chlorinated paraffin wax

chlorinated petroleum

chlorinated aliphatic fractions of mineral oil

II. Amines, e. g.

Primary, secondary, and tertiary, e. g.

fluorinated tri-butyl amines

fluorinated tri-allyl amines

fluorinated hexyl amines

III. Nitriles, e. g.

Chlorinated or fluorinated

ethyl cyanide

butyl cyanide

octyl cyanide

lauryl nitrile

stearyl nitrile

The halogen bearing compounds which may thus be advantageously employed in combination with the sulphur compounds of the type above identified may also desirably contain oxygen and such halogen and oxygen bearing organic compounds may be classified as follows:

*Halogen and oxygen-bearing organic ring compounds*

Oxygen-bearing derivatives of:

A. "Carbon ring" type compounds

(1) of the aromatic, or allied type, including oxygen-bearing derivatives of benzene, naphthalene, anthracene, etc., also compounds of the bridged ring type, such as the terpenes, and related compounds.

(2) of the class including the cycloparaffins, cyclo-olefines, etc. Examples of this class are oxygen-bearing derivatives of the following:

(a) Hydrogenation products of benzene (e. g. cyclohexane, cyclohexene, cyclohexadiene), such as hydrogenated phenol, notably cyclohexanol di-hydro phenol tetra-hydro phenol

(b) Hydrogenation products of naphthalene (e. g., decahydronaphthalene, tetra-hydronaphthalene, etc.), such as the hydrogenated naphthols.

(c) Naphthenes, such as naphthenic acid, etc.

(3) of mixed type such as derivatives of indene, hydrindene, hydranthracene, etc.

B. "Heterocyclic" type compounds

(1) of the aromatic or allied type including derivatives of pyridine, quinoline, etc.

(2) other types such as furane and its derivatives and derivatives of thiophene, pyrrole, etc.

*Halogen and oxygen-bearing aliphatic compounds*

Alcohols (mono-, di-, and tri-hydric) e. g.

ethylene chlorhydrin glycerol monochlorhydrin fluorinated octyl alcohol fluorinated decyl alcohol fluorinated lauryl alcohol chlorinated octadecyl alcohol

Esters and salts, e. g.

methyl chlorpropionate ethyl chlorlaurate methyl dichlorstearate chlorinated mono- and di-glycol esters of propionic, lauric, and stearic acids chlorinated mono-, di-, and tri-glycerol esters of propionic, lauric, and stearic acids methyl dichlorpalmitate sodium chlorhydroxy stearate calcium di-chloro stearate aluminum di-chloro stearate

Ethers, e. g.

chloromethyl propyl ether chlor butyl ether chlor amyl ether chlor methyl lauryl ether

Ketones, e. g.

chloromethyl ethyl ketone chlor dibutyl ketone chlor palmitone chlor laurone chlor stearone

Aldehydes, e. g.

chlorbutanal chlorpentanal

Acids, e. g.

chlorpropionic acid chlorauric acid chlormyristic acid chlorpalmitic acid chlorstearic acid chlorricinoleic acid chlor crotonic acid chlor acrylic acid chlor oleic acid

Other halogen containing compounds which may be employed to advantage in lubricating compositions along with the previously identified sulphur compounds are as follows:

Halogenated aliphatic phosphorus-containing compounds

chlor-lauryl phosphine chlor-octyl phosphine chlor-di-ethyl di-thiophosphine sulfide chlor-amyl phosphite chlor-butyl phosphate chlor-lauryl phosphite chlor-lauryl thiophosphate chlor-lauryl thiophosphite

Halogenated aliphatic compounds containing sulfur and nitrogen

chlor-lauryl thiocyanide

chlor-butyl thiocyanate

Halogenated aliphatic compounds containing sulfur

chlor-amyl sulfide

chlor-butyl disulfide

While the above compounds have been disclosed primarily as separate halogen compounds which

may be used in conjunction with our thiocarbonates, they may also serve another use. Many of them may be used to react with alkali metal thiocarbonates to form the substituted thiocarbonates which are the principal products of our invention.

For these secondary uses, the halogen in these compounds may be replaced in whole or in part. It will be obvious to those skilled in the art that most of these compounds are useful only in introducing the second R of our thiocarbonates since the first is derived from an alcoholic compound, carbon disulfide and a caustic metal hydroxide. Furthermore it will be obvious that in order to come within the scope of our claims the halogenated hydrocarbons listed above may be used only with such alkali thiocarbonates as contain in the first R group one of the characterizing elements.

Our addends are admirably adapted for use in lubricating oils of all types including those designed for use in automotive crankcases, Diesel oils, and any other oils of lubricating viscosity.

Certain lubricating compositions containing certain of the addition agents above mentioned will be found particularly useful in the lubrication bearings formed of cadmium or lead containing bearing metals such as, for example, cadmium-silver and copper-lead bearings. Furthermore, our addends are advantageously blended in gasoline and other petroleum fuels either directly or after being blended first in a lubricating oil and then added to the fuel. Soap-thickened mineral oils of all types ranging from those showing only a slight increase in viscosity over that of the mineral oil alone to the semi-solid and solid greases containing fifty per cent or more of soap are amenable to treatment according to our invention. In making these greases, the usual soaps such as sodium stearate, aluminum stearate, calcium soaps of beta fat, and the like may be used to form the large part of the necessary soap. Various other thickening ingredients or materials for other purposes may be added. These include yarn, hair, graphite, glycerol, water, lampblack, mica, zinc, dust, litharge, and the like.

In making a lubricating gasoline, we blend 0.5 per cent of the product of Example 19 with gasoline. It is to be understood, however, that the hydrocarbon oil in the treated fuels may be of a viscosity of from about 35 seconds at 100° F. S. S. U. to 350 seconds or more and the amount of oil blended with the thiocarbonate to form the fuel addend may vary between 0% to 99.5%.

In some cases the fuel may be prepared without adding any hydrocarbon oil. The quantity of thiocarbonate in the final blended fuel may vary from 0.0001 to 1.0% or slightly more.

It will be understood that certain features and sub-combinations may be employed without reference to other species or combinations. This is contemplated by and is within the scope of our claims. It is further obvious that various changes may be made in details within the scope of our invention. It is therefore to be understood that our invention is not to be limited to the details described.

This application is a continuation-in-part of our copending application Serial No. 298,337, filed October 6, 1939, now Patent No. 2,368,670 dated February 6, 1945.

Other modes of applying the principle of the invention may be employed, change being made as regards the details described, provided the fea-

tures stated in any of the following claims or the equivalent of such be employed.

We therefore particularly point out and distinctly claim as our invention:

1. A lubricant comprising in combination a major amount of oil of lubricating viscosity and from 0.001% to 10% of an oil-soluble neutralized organic carboxylic acid bearing a thiocarbonate radicle having the formula:



where C represents carbon; X is an element selected from the class consisting of oxygen and sulphur, at least one X is sulphur; Y is a halogen; R is an organic radicle; and Q is one hydrogen equivalent of a sole-forming radicle.

2. A lubricant comprising in combination a major amount of oil of lubricating viscosity and from 0.001% to 10% of an oil-soluble compound having the formula:



in which C represents carbon; X is an element selected from the class consisting of oxygen and sulphur, at least one X is sulphur; Y is a halogen; R is an organic radicle, and Q' is a radicle containing trivalent nitrogen.

3. A lubricant comprising in combination a major amount of oil of lubricating viscosity and from 0.001% to 10% of an oil-soluble compound having the formula:



in which C represents carbon; X is an element selected from the class consisting of oxygen and sulphur, at least one X is sulphur; Y is a halogen; R is an organic radicle; and Q'' is a radicle containing pentavalent nitrogen.

4. A lubricant comprising in combination a major amount of an oil of lubricating viscosity and a minor amount, sufficient to improve the extreme pressure characteristics of the oil, of an oil soluble neutralized organic carboxylic acid bearing a thio-carbonate radicle having the formula:



where C represents carbon; X is an element selected from the class consisting of oxygen and sulphur, at least one X is sulphur; Y is a halogen; R is an organic radicle; and Q is one equivalent of a metal.

5. A composition in accordance with claim 1 in which Q is one equivalent of a non-metallic salt-forming radicle.

6. A composition in accordance with claim 1 in which Q is one equivalent of an organo-metallic radicle.

7. A composition in accordance with claim 1 in which at least one X in the grouping



is sulphur.

10 8. A composition in accordance with claim 1 in which Q is an organo-metallic radicle and at least one X in the grouping



15 is sulphur.

9. A composition in accordance with claim 1 in which at least two X's in the grouping



20 are sulphur.

10. A composition in accordance with claim 1 in which Q is an organo-metallic radicle and at least two X's in the grouping



are sulphur.

11. A composition in accordance with claim 1 in which at least 3 X's in the grouping



are sulphur.

12. A composition in accordance with claim 1 in which Q is an organo-metallic radicle and at least 3 X's in the grouping



40 are sulphur.

13. A composition in accordance with claim 1 in which R is aliphatic.

14. A composition in accordance with claim 1 in which R is aliphatic and Q is an organo-metallic radicle.

BERT H. LINCOLN.  
GORDON D. BYRKIT.

#### REFERENCES CITED

The following references are of record in the file of this patent:

#### UNITED STATES PATENTS

| 55 | Number    | Name           | Date          |
|----|-----------|----------------|---------------|
|    | 2,153,496 | Berger         | Apr. 4, 1939  |
|    | 2,158,668 | Rosen          | May 16, 1939  |
|    | 2,197,835 | Reiff          | Apr. 23, 1940 |
|    | 2,257,750 | Lincoln        | Oct. 7, 1941  |
| 60 | 2,288,288 | Lincoln        | June 30, 1942 |
|    | 2,289,795 | McNab          | July 14, 1942 |
|    | 2,320,287 | Lieber         | May 25, 1943  |
|    | 2,365,011 | Rosen          | Dec. 12, 1944 |
| 65 | 2,368,670 | Lincoln et al. | Feb. 6, 1945  |
|    | 2,369,150 | Lincoln et al. | Feb. 13, 1945 |